



The steel of such analysis is worked into sheet and strip form by the usual hot mill methods, or hot and cold mill methods, to a gauge usually in the order of .014". The final gauge is not critical.

The sheets and strip are then normalized for strain removal and recrystallization in a continuous furnace containing an atmosphere of CO<sub>2</sub> of from 8 to 15%, water vapor of from 1 to 3.5% (or sufficient to saturate the total atmosphere at temperatures from 50° F. to 85° F.), and the balance, by difference, principally of nitrogen, with a usual total impurity content in the neighborhood of 3%, mainly of carbon monoxide, hydrogen, and methane. This atmosphere corresponds to that disclosed in my prior application referred to above, and is effective at temperature to provide mildly oxidizing conditions in the furnace.

I have discovered that when silicon electrical steels are aluminized to such an extent as to contain from .10% to 1.00% aluminum, the desired extent of recrystallization and grain growth may be obtained at temperatures of from 1500° F. to 1750° F., the time factor varying inversely with the temperature. For the greatest time/temperature economy, I have found that a temperature in the neighborhood of 1750° F. will develop electrical properties of watt loss ranging from 0.60 watt/lb. for a time in the furnace of 1½ minutes, down to less than 0.50 watt/lb. for a time in the furnace of 6 minutes. In accordance with the method of the present invention, a steel containing 3.51% silicon and about 0.30% aluminum, having a watt loss value as low as 0.450 watt/lb., has been made by heating in the neighborhood of 1750° F. for 6 minutes in the atmosphere here prescribed.

It will be appreciated that these exceptional electrical properties are stabilized by annealing, after the heat treatment above described, at a temperature usually around 1425° F. for a few hours. The stabilizing anneal is susceptible of considerable variation as to time and temperature, having been successfully applied at temperatures of from 1300° F. up to 1600° F., and for periods of time ranging between one-half to six hours. This stabilization anneal is accompanied by a further lowering of the watt loss values, and has yielded a product having a watt loss rating of substantially .40 watt/lb. All of the values herein cited are for an induction of 10,000 gaussess at 60 cycles.

It will be understood that the steels contemplated for treatment hereby may, in addition to the silicon, aluminum, and carbon contents prescribed, contain usual amounts of other elements common in steels of the type, such as, manganese up to 0.40%, and phosphorus and sulphur each around 0.010%. Small amounts of other elements are admissible.

It will be understood that the steel may be worked or cold worked to gauge, or both, the usual practice being to roll hot strip continuously to around .062" gauge, and, then, cold reduce it continuously in strip form to gauges ranging between .014" and .022". The final thickness will determine the rapidity of response of the material to heat treatment, and prescribe the manner of heat treatment as between continuous and batch methods. Beyond this, however, the ultimate gauge thickness, and the form of the heat treatment, are not critical.

Similarly, the sheets and strip may be hot worked or cold worked to gauge, or both, the usual practice being to roll hot strip continuously to around .062" gauge, and, then, cold reduce it continuously in strip form to gauges ranging between .014" and .022". The final thickness will determine the rapidity of response of the material to heat treatment, and prescribe the manner of heat treatment as between continuous and batch methods. Beyond this, however, the ultimate gauge thickness, and the form of the heat treatment, are not critical.

This application is a continuation of my pending application bearing Serial No. 460,001, now abandoned, which was filed September 28, 1942, and which was a continuation-in-part of the application which matured into Patent No. 2,304,518, and is also a continuation of my patent application Serial No. 584,257, now abandoned, filed March 22, 1945.

While I have shown and described certain specific embodiments of the present invention, it will be readily understood by those skilled in the art that I do not wish to be limited exactly thereto, since various modifications may be made without departing from the scope of the invention as defined in the appended claim.

I claim:

A method of making aluminized silicon steel electrical strip or sheet; said method comprising the steps of producing an aluminized silicon steel with a composition suitable for said product and containing from 1% to 5% silicon, from .10% to 1.00% aluminum and substantially more than about .02% carbon; working said steel to strip or sheet, and continuously annealing said strip or sheet in a decarburizing atmosphere at temperatures of from 1500° F. to 1750° F. to reduce the carbon to less than .02%, said atmosphere being oxidizing to a degree regulated to cause the formation of a thin, tightly adherent oxide film on said strip or sheet without the production of a heavy, loose scale and consisting of from 8% to 15% carbon dioxide with the balance mainly nitrogen and sufficient water to saturate said atmosphere with water vapor at from 50° to 85° F.

ALVIN R. WILLIAMS.

#### REFERENCES CITED

50 The following references are of record in the file of this patent:

#### UNITED STATES PATENTS

Number Name Date  
55 2,304,518 Williams Dec. 8, 1942

#### OTHER REFERENCES

"Alloys of Iron and Silicon," Griener et al., pages 385 and 386, McGraw-Hill Book Co., N. Y., 1933.